

3,301,690

PRODUCTION OF DIRECT BONDED BASIC BRICK  
George R. Rigby, Lachute, Quebec, Canada, assignor to  
Canadian Refractories Limited, Montreal, Quebec,  
CanadaNo Drawing. Filed Aug. 27, 1964. Ser. No. 392,617  
Claims priority, application Great Britain, Aug. 29, 1963,  
34,302/63

1 Claim. (Cl. 106—59)

This invention relates to the manufacture of direct bonded basic brick.

A typical basic refractory brick for use, for instance, in open hearth roof construction, comprises 80% graded magnesia ( $MgO$ ) and 20%  $-4 +10$  mesh (Tyler standard) chrome ore.

Normally, basic brick, containing most or all of the chrome ore fraction as coarse grains have, after firing, a gap around the chrome grains which, therefore, fit loosely into the brick matrix. This gap is produced by the partial dissolution of the chrome spinel constituents in the surrounding magnesia matrix during initial firing. Furthermore, the silicate gangue associated with the chrome ore melts and then distributes itself around the chrome grains as a silicate "halo" or fringe on the matrix side of the gap.

It is well known that open hearth roof brick absorb both iron oxide ( $Fe_2O_3$ ) and lime ( $CaO$ ) at the hot face in service and these migrate back into the brick, the lime silicates migrating farther behind the hot face than the  $Fe_2O_3$  where they freeze and concentrate in zones. With a conventional brick containing both a gap and silicate "halo" around the chrome grains, there is a mechanism of failure in which, firstly, the silicate halo melts and migrates after combination with either the absorbed  $Fe_2O_3$  or  $CaO$  and, since this is already associated with a gap, the space between the chrome grains and matrix is further widened. This eventually creates a series of channels through the brick along which  $Fe_2O_3$  and silicates can migrate readily. As they migrate,  $MgO$  is dissolved making these channels larger until they take the form of conspicuous voids located a short distance behind the hot face. The next stage is for these voids to be linked together by means of horizontal cracks, and the final stage is for the face of the brick to drop off as a peel which is so often observed in basic brick that have absorbed molten slags. It is, therefore, desirable, in order to increase service life, that the silicates in the brick should be kept at a minimum and should be distributed throughout the brick and not concentrated in the most vulnerable areas around the chrome grains. Moreover, it is desirable that any gaps around the chrome grains should be dispersed so that no preferential channels are established as a result of absorption and migration of liquid slag.

The invention resides in a magnesite chrome refractory brick comprising 5-40% particles of chrome ore containing not more than about 5%  $SiO_2$  and having a particle size of  $-4 +28$  mesh, granular magnesia containing not more than 1%  $Fe_2O_3$ , 2%  $CaO$ , and 2%  $SiO_2$  and having a particle size of  $-4$ , and 5-40% particles of a clinker having a particle size of  $-65$  mesh and being a fired homogeneous mixture of magnesia and 5 to 15% of a crystal growth promoting agent selected from the group consisting of chrome ore, iron oxide, titanium dioxide, and chromium oxide.

The invention also resides in a method of making magnesite chrome refractory brick which comprises forming a clinker by firing to a temperature to form a homogeneous solution, a mix consisting essentially of magnesia and 5 to 15% of a material selected from the group consisting of chrome ore, iron oxide, titanium dioxide, and

chromium oxide, grinding said clinker to particles of  $-65$  mesh, forming a brick mixture consisting essentially of 10-40% particles of chrome ore containing not more than 5%  $SiO_2$  and having a particle size of  $-4 +28$  mesh, granular magnesia containing not more than 2%  $CaO$  and 2%  $SiO_2$  and having a particle size of  $-4 +65$  mesh, and 10 to 40% of said clinker particles, pressing said mixture into shapes, and firing said shapes at a temperature of about  $1600^{\circ} - 1700^{\circ} C$ .

10 In accordance with the invention, most or all of the fines ( $-65$  mesh) portion of the conventional brick is replaced with a special clinker made by firing at least to a temperature to obtain chemical homogeneity, a mixture of magnesia and 5% to 15% of a crystal growth promoting agent. The clinker is cooled and ground to at least  $-65$  mesh (Tyler standard).

15 Crystal growth promoting agents of the type employed are partially soluble in magnesia, so that the special clinker is a homogeneous solid solution at high temperatures, although at room temperatures there may be a microscopically disseminated precipitate of a separate phase with a spinel structure.

20 When a brick is made, the fines of the brick mix fill the interstices around the coarse and intermediate grains. Thus, each coarse chrome grain is surrounded by the fine clinker which, upon firing, recrystallizes to form larger magnesia crystals. This crystal growth disrupts the edges of the  $MgO$  grains, detaching individual periclase crystals, which, because of the expansion and 25 30 loosening of the  $MgO$  grain texture, move across the gap and attach themselves to the surface of the chrome grains.

35 Direct bonding, therefore, is assisted by promoting the solution of spinels into the  $MgO$  which, in turn, is promoted by high firing temperatures.

40 While the agent employed in the pre-sintering step may be iron oxide ( $Fe_2O_3$ ), chromium oxide ( $Cr_2O_3$ ), titanium dioxide ( $TiO_2$ ), or fine chrome ore, the most suitable ones are  $Fe_2O_3$  and finely divided chrome ore. About 5% to 15% by weight of such agent is used in forming the special clinker.

45 The discontinuous nature of a brick structure produces spalling resistance. When the fine crystals composing the magnesia grains being to grow, grain boundaries tend to disappear and the discontinuous structure, and, therefore, spalling resistance, is lost.

50 The agents used in preparing the special clinker act so effectively to promote grain growth, that it is important to have them present only in the fines. The coarse and intermediate size of magnesia grains should be of high purity, low particularly in the oxides, of chromium, titanium, iron, and silicon. They will then retain their identity throughout the service life of the brick, at least until the iron oxide pick-up reaches them.

55 As previously indicated, it is desirable that the silica ( $SiO_2$ ) content of the brick be kept at a minimum. Since magnesias with very low silica contents are readily available nowadays, the  $SiO_2$  is largely contributed by the chrome ore. Thus, it is desirable to utilize chrome ore containing not more than 5% and preferably not more than 2% and to maintain the chrome ore content at the lowest effective level. Such  $SiO_2$  as remains should be dispersed as widely as possible throughout the brick and this is attained by high firing temperatures which

60 65 cause the silicates to migrate away from the chrome grains further into the magnesia matrix so that the silicate "halo" is dispersed. This is a second reason why high firing temperatures are desirable. The chrome ore is graded  $-4 +10$  mesh (Tyler standard). Coarse chrome ore is

70 considered essential since this is the constituent of the brick which retains its identity longest and maintains spalling resistance during service.

The magnesia used in the mix should contain not more than 1%  $Fe_2O_3$ , 2%  $CaO$ , and 2%  $SiO_2$  and has a particle size of  $-4 +65$  mesh (Tyler standard).

The brick mix comprises 10% to 40% of chrome ore, magnesia, and 10% to 40% clinker, of the specified characteristics. It will be apparent that the size grading of the brick mix is about the same as used in conventional brick making; that is, using about 30-40% of  $-65$  mesh material.

Normally a binder, such as waste sulfite liquor or Epsom salts, is used in the mix primarily to impart sufficient strength to the brick shapes to permit handling of the same between the pressing and firing operations. Such binders usually either disappear during firing or leave such little residuum as to have no effect on the behaviour and properties of the brick.

The brick is pressed in a conventional refractory brick making press and fired at a temperature of  $1600^{\circ}$  to  $1700^{\circ}$  C., and preferably about  $1650^{\circ}$  C.

While not intended to be limitative, the following procedure may be followed in forming the mix:

The coarse chrome ore is initially charged into the mixer and then sufficient binder to coat it. Next, the special clinker powder is added in sufficient quantity to coat the chrome ore grains. Finally, the coarse magnesia, the rest of the binder, and fine magnesia are added. In this instance, only a portion of the fines comprises the special clinker powder. Thus, by following this procedure, not only is the special clinker powder placed adjacent the coarse chrome grains only, but the quantity required of such powder is lessened.

The brick produced in accordance with the invention as compared with conventional brick, has an increased modulus of rupture, and an increased modulus of elasticity, both at room and elevated temperatures.

The following examples are illustrative of the invention. The magnesia employed was the same in all instances and contained not more than 1%  $Fe_2O_3$ , 2%  $CaO$ , and 2%  $SiO_2$ . The chrome ore employed was also the same in all instances and contained not more than 5%  $SiO_2$ .

#### Example I

A clinker was made from 10%  $Fe_2O_3$  and 90% magnesia. After cooling, it was ground to at least  $-65$  mesh. A brick mix was made containing:

|                           | Percent |
|---------------------------|---------|
| $-10 +28$ mesh chrome ore | 20      |
| $-4 +65$ mesh magnesia    | 40      |
| $-65$ mesh clinker        | 40      |

A small amount of binder (not more than 5% of the total mix) and consisting of waste sulfite liquor was employed as the binding agent for the shapes before firing.

The mix was pressed into shapes and fired in conventional manner at a temperature of about  $1650^{\circ}$  C.

#### Example II

This example is the same as Example I except that the clinker was made from 10% chrome ore and 90% magnesia.

#### Example III

This example was conducted for comparison purposes and followed the conditions of the other examples except that the brick mix was conventional, as follows:

|                           | Percent |
|---------------------------|---------|
| $-10 +28$ mesh chrome ore | 20      |
| $-4 +65$ mesh magnesia    | 40      |
| $-65$ mesh magnesia       | 40      |

Thin sections of brick made by each of the examples were measured petrologically for direct bonding characteristics. Each of the sections from Example I and II showed well developed direct bonding in that the periclase crystals were attached to the chrome grains along the border thereof. The sections of brick made by Example III showed only slight attachment of magnesia crystals to some chrome grains with most of the chrome grains having gaps around them.

A modulus of rupture test at a temperature of  $1250^{\circ}$  C., which is sometimes employed as an indication of direct bonding development, had the following results:

Example I—310 p.s.i.  
Example II—310 p.s.i.  
Example III—140 p.s.i.

These tests were made on one inch square bars. It will be apparent that higher but still relative values would be obtained when testing bricks of full size.

A cold modulus of rupture test had the following results:

Example I—440 p.s.i.  
Example II—450 p.s.i.  
Example III—410 p.s.i.

The screen sizes given throughout this specification and accompanying claim are Tyler standard.

I claim:

A method of making magnesite chrome refractory brick which comprises the successive steps of mixing a binder with a quantity of particles of chrome ore containing not more than 5%  $SiO_2$  and having a particle size of  $-4 +28$  mesh to coat said particles with said binder, mixing with said binder-coated particles a quantity of particles of clinker having a particle size of  $-65$  mesh to coat said binder-coated particles with said clinker particles, said clinker having been formed by firing a mixture consisting essentially of magnesite and 5% to 15% of a material selected from the group consisting of chrome ore, iron oxide, titanium dioxide, and chromium oxide at a temperature to obtain chemical homogeneity thereof, forming a mixture consisting essentially of said clinker-coated particles and an additional quantity of binder and a quantity of magnesia particles containing not more than 1%  $Fe_2O_3$ , 2%  $CaO$ , and 2%  $SiO_2$ , and having a particle size of  $-4 +65$  mesh, said mixture containing 5-40% of said chrome ore particles, 5-40% of said clinker particles, and the balance said magnesia particles, pressing said mixture into shapes, and firing said shapes at a temperature of  $1600^{\circ}$ - $1700^{\circ}$  C.

#### References Cited by the Examiner

##### UNITED STATES PATENTS

60 3,180,743 4/1965 Davies et al. ----- 106-59  
3,210,206 10/1965 Davies et al. ----- 106-59

HELEN M. McCARTHY, Acting Primary Examiner.

65 TOBIAS E. LEVOW, J. E. POER, Assistant Examiners,